# EUROPEAN PATENT SPECIFICATION

(11) **EP 3 795 711 B1**
(45) Date of publication and mention of the grant of the patent: **07.02.2024**
(21) Application number: 18924969.1
(22) Date of filing: 12.09.2018
(51) Int. Cl.: C22C 38/50, C22C 38/48, C22C 38/42, C22C 38/06, C22C 38/04, C22C 38/02, C22C 38/00, C21D 6/00, C21D 1/26, C21D 9/46

(54) **LOW CR FERRITIC STAINLESS STEEL HAVING EXCELLENT DAMPING CAPACITY AND MANUFACTURING METHOD THEREFOR**
NIEDRIG CR-LEGIERTER ROSTFREIER FERRITISCHER STAHL MIT AUSGEZEICHNETER DÄMPFUNGSKAPAZITÄT UND VERFAHREN ZU SEINER HERSTELLUNG
ACIER INOXYDABLE FERRITIQUE À FAIBLE TENEUR EN CR PRÉSENTANT UNE EXCELLENTE CAPACITÉ D'AMORTISSEMENT ET SON PROCÉDÉ DE FABRICATION

(30) Priority: 26.06.2018 KR 20180073250
(43) Date of publication of application: 24.03.2021
(73) Proprietor: POSCO Co., Ltd, Pohang-si, Gyeongsangbuk-do 37859 (KR)
(72) Inventor: JUNG, Il Chan, Pohang-si, Gyeongsangbuk-do 37665 (KR); RYU, Sung Hee, Seoul 06000 (KR); LEE, Kye-Man, Seoul 02798 (KR)
(74) Representative: Potter Clarkson
(86) International application number: PCT/KR2018/010699
(87) International publication number: WO 2020/004710

(56) References cited:
- WO-A1-2018/181060
- CN-A- 102 234 740
- CN-A- 102 234 740
- JP-A- 2009 299 182
- JP-A- 2009 299 182
- JP-A- 2010 070 799
- KR-A- 20160 077 515
- KR-B1- 101 762 046
- US-A1- 2014 023 550
- KOBAYASHI et al.: "Effect of Nb Addition on Cu Precipitation in Ferritic Stainless Steel", ISIJ international, vol. 51, no. 4, 2011, pages 657-662, XP055666762,

## Description

### [Technical Field]

The present disclosure relates to a low-Cr ferritic stainless steel with excellent vibration attenuation ability to absorb external vibration energy and a manufacturing method thereof.

### [Background Art]

Ferritic stainless steel has excellent corrosion resistance while adding less expensive alloying elements, and has a higher price competitiveness than austenitic stainless steel. In particular, 9-14% of low-Cr ferritic stainless steel has superior cost competitiveness and is used in exhaust system parts (Muffler, Ex-manifold, Collector cone, etc.) corresponding to the exhaust gas temperature range of room temperature to 800°C. The steel plate for vehicle exhaust system must be capable of absorbing noise and vibration generated during engine or other driving, and must be able to withstand external environmental factors such as exhaust gas generated inside the vehicle, rain or fog. Therefore, sound absorption and corrosion resistance must be secured.

In order to solve this problem, in the case of high Cr ferritic stainless steel, attempts have been made to improve the vibration attenuation ability by controlling the number of precipitates, solid solution C, N, and the size and shape of inclusions, and the effects have been reported. However, there are no attempts and achievements to improve vibration attenuation ability by specializing in low-Cr ferritic stainless steel.

JP 2009 299182 A discloses a ferritic stainless steel containing, by mass, C: 0.03% or less, Si: 3% or less, Mn: 2% or less, P: 0.05% or less, S: 0.03% or less, Cr: 11 to 30%, Nb: 0.15 to 0.8%, and N: 0.03% or less, with the remainder comprising Fe and unavoidable impurities, and for which the value A is 0.10 to or higher when A=Nb-(C×92.9/12+N×92.9/14).

KR 2016 0077515 A discloses a high corrosion resistance steel sheet with excellent sound absorption, and a manufacturing method thereof. The high corrosion resistance steel sheet with excellent sound absorption comprises: 0.005-0.01 wt% of carbon (C), 0.005-0.01 wt% of nitrogen (N), 0.3 wt% or less of silicon (Si) (excluding 0 wt%), 0.5 wt% or less of manganese (Mn) (excluding 0 wt%), 0.001-0.035 wt% of phosphorus (P), 0.001-0.01 of sulfur (S), 0.1 wt% or less of titanium (Ti) (excluding 0 wt%), 0.1 wt% or less of niobium (Nb) (excluding 0 wt%), 0.1 wt% or less of aluminum (Al) (excluding 0 wt%), 16.0-22.0 wt of chromium (Cr); and the remaining consisting of iron (Fe) and unavoidable impurities, satisfying equations (1) and (2), wherein equation (1): 0.008<=(C+N)(ppm)<=0.018 and equation (2): (Ti+Nb+AI)(wt%)<0.01.

US 2014/023550 A1 discloses a ferritic stainless steel sheet which exhibits characteristic heat resistance at 950° C. and workability at ordinary temperature, and that contains, by mass %, C: 0.02% or less, N: 0.02% or less, Si: over 0.1 to 1.0%, Mn: 0.5% or less, P: 0.020 to 0.10%, Cr: 13.0 to 20.0%, Nb: 0.5 to 1.0%, Cu: 1.0 to 3.0%, Mo: 1.5 to 3.5%, W: 2.0% or less, B: 0.0001 to 0.0010%, and AI: 0.01 to 1.0% and a balance of Fe and unavoidable impurities, and where Mo+W is 2.0 to 3.5%.

### [Disclosure]

### [Technical Problem]

The present invention provides a low-Cr ferritic stainless steel and a manufacturing method thereof maximizing the vibration attenuation ability by utilizing the Nb, Cu fine precipitated phase.

### [Technical Solution]

The invention is as specified in the appended claims.

### [Advantageous Effects]

The low-Cr ferritic stainless steel according to the invention increases vibration attenuation ability by 100% or more through a sound absorption mechanism by the movement of solid solution C and N and a vibration attenuation mechanism through suppression of precipitation of carbonitrides.

In addition, the low-Cr ferritic stainless steel according to the invention has excellent corrosion resistance, so that when used in vehicle exhaust system parts, etc., quietness and durability can be secured.

### [Description of Drawings]

FIG. 1 is a graph showing the correlation of the vibration attenuation index according to the number of Nb Laves phase precipitates and Cu precipitates.
FIG. 2 is a photograph showing the distribution of Nb Laves phase precipitates and Cu precipitates at the matrix interface.

### [Best Mode]

A low-Cr ferritic stainless steel with excellent vibration attenuation ability according to the invention includes, in percent (%) by weight of the entire composition, C: 0.005 to 0.01%, N: 0.005 to 0.01%, Si: 0.1 to 0.9%, Mn: 0.1 to 0.9%, Cr: 9 to 14%, Ni: 0.3% or less, P: 0.04% or less , S: 0.002% or less, Ti: 0.15 to 0.3%, Nb: 0.15 to 0.3%, Cu: 0.15 to 0.3%, Al: 0.01 to 0.05%, the remainder of iron (Fe) and other inevitable impurities, and includes 5×10²/ mm² or more of Nb laves phase precipitates and Cu precipitates, , wherein the content of C+N is less than or equal to 0.02%; and wherein a vibration attenuation index (Q- 1) of the stainless steel is 2.0×10⁻⁴ or more at 25°C, 2.5×10⁻⁴ or more at 300°C..

The ferritic stainless steel according to an embodiment of the invention satisfies the following equation (1). $\left(Nb+Cu\right) / Ti \geq 1.5$

Here, Nb, Cu, Ti mean the content (% by weight) of each element.

### [Modes of the Invention]

The present inventors have conducted various studies in order to improve the vibration attenuation ability of low-Cr ferritic stainless steel, and have obtained the following knowledge.

The sound-absorbing mechanism (Snoek Effect) indicates that during vibration, solid solution C and N cause energy loss while changing their position in the lattice, and as a result, absorb sound. The sound-absorbing effect by solid solution C and N is proportional to the amount of solid solution C and N, and the vibration attenuation effect by magnetic domain wall becomes better as there are no factors that hinder the movement of the magnetic domain wall such as precipitate, dislocation, and internal stress.

In general, a trace amount of Ti and Nb is added to the ferritic stainless steel for exhaust system for corrosion resistance of the weld. In the case of such ferritic stainless steel with Ti and Nb added, a large amount of Ti(C,N) and Nb(C,N) carbonitrides are inevitably precipitated in the ferrite matrix of the surface layer. These Ti(C,N), Nb(C,N) precipitates are essentially inferior in the vibration attenuation ability of ferritic stainless steel because they inhibit the movement of the magnetic domain wall, which is one of the vibration attenuation mechanisms during vibration. In addition, since C and N are mostly combined with Nb and Ti in a precipitate state, there is relatively no solid solution C and N present in the ferrite matrix. Therefore, the sound absorption mechanism (Snoek Effect) due to the movement of solid solution C and N during vibration cannot be expected.

On the other hand, Nb is added for high temperature strength to ferritic stainless steel that is applied at high temperatures of 400°C or higher, and Cu is added as a solid solution strengthening element. In this case, a fine-sized Nb Laves Phase (Fe₂Nb) and Cu precipitated phase of 1 to 200 nm may be generated under specific heat treatment conditions, the interface between the coherent precipitated phase and the matrix reacts to external vibration and vibrates together, and by absorbing external vibration energy, the vibration attenuation ability can be increased. At this time, the effect is further increased when the Nb Laves phase or Cu is precipitated in a complex manner than when precipitated alone. However, when the size of the precipitate is coarsened to more than 200 nm, the coherency of the precipitate and the matrix decreases, and the number of precipitates decreases, so the effect of improving the vibration attenuation ability is rather offset. Therefore, the vibration attenuation ability can be maximized by precipitating fine Nb Laves-phase precipitates and Cu precipitates at the interface of the matrix.

A low-Cr ferritic stainless steel with excellent vibration attenuation ability according to the invention includes, in percent (%) by weight of the entire composition, C: 0.005 to 0.01%, N: 0.005 to 0.01%, Si: 0.1 to 0.9%, Mn: 0.1 to 0.9%, Cr: 9 to 14%, Ni: 0.3% or less, P: 0.04% or less , S: 0.002% or less, Ti: 0.15 to 0.3%, Nb: 0.15 to 0.3%, Cu: 0.15 to 0.3%, Al: 0.01 to 0.05%, the remainder of iron (Fe) and other inevitable impurities, and includes 5×10²/ mm² or more of Nb laves phase precipitates and Cu precipitates, wherein the content of C+N is less than or equal to 0.02%; and wherein a vibration attenuation index (Q- 1) of the stainless steel is 2.0×10-⁴ or more at 25°C, 2.5×10⁻⁴ or more at 300°C..

Hereinafter, the reason for the numerical limitation of the content of the alloy component element in the present disclosure will be described Hereinafter, unless otherwise specified, the unit is% by weight.

The content of C is 0.005 to 0.01%.

C is a key element that causes sound absorption, and since the solid solution C continues to move from its original position in the lattice of the matrix to another position when the steel plate vibrates, energy loss occurs and sound absorption occurs. In general, as the solid solution C in the matrix increases, the sound absorption and vibration attenuation ability increases. However, when the content exceeds 0.01%, the concentration of solid solution C reaches its limit, and it combines with Cr to form Cr₂₃C₆ precipitates, which hinders the movement of the magnetic domain wall, and local Cr depletion within the matrix causes golden dust. Therefore, corrosion resistance is lowered.

The content of N is 0.005 to 0.01%.

Among the steels, N is a key element that causes sound absorption and vibration attenuation through the same mechanism as C. As the solid solution N in the matrix increases, the vibration attenuation ability increases. However, if it exceeds 0.01%, the concentration of solid solution N reaches its limit, it binds to Cr and generates Cr₂N precipitates, which hinders the movement of the magnetic domain wall, and local Cr depletion within the matrix causes golden dust. Therefore, corrosion resistance is lowered.

The precipitation of carbonitrides can be suppressed by increasing the solid solution C and N in the matrix by controlling the content of C+N to be less than or equal to 0.02%, and the vibration attenuation ability due to the smooth movement of the magnetic domain wall can be improved.

The content of Si is 0.1 to 0.9%.

Si is an element that acts as a deoxidizer in steel making, and contains 0.1% or more. However, when it is contained in a large amount, inclusions are generated due to Si oxide, and since such inclusions hinder the movement of the magnetic domain wall and thus inhibit vibration attenuation ability, the content is limited to 0.9% or less.

The content of Mn is 0.1 to 0.9%.

Mn serves to stabilize austenite. When it is contained in a large amount, the austenite-ferrite transformation point (Ac1) is lowered, and high temperature annealing capable of dissolving C and N after cold rolling becomes impossible, so the content is limited to 0.9% or less.

The content of Cr is 9 to 14%.

Cr increases the magnetostriction constant of the steel to further promote the movement of the magnetic domain wall compared to carbon steel when vibration occurs, and increases the vibration attenuation ability by the movement of the magnetic domain wall. It also plays a positive role in the vibration attenuation effect caused by C and N. However, if the Cr content exceeds 14%, because carbonitrides are easily formed by easily combining with C and N, the amount of solid solution C and N is lowered, and the precipitate interferes with the movement of the magnetic domain wall. Therefore the content is limited to the above range..

The content of Ni is 0.3% or less.

Ni may be contained in an amount of 0.1% as an impurity unavoidably included in steel by scrap melting, and its upper limit is 0.3%.

The content of P is 0.04% or less.

P is an inevitable impurity contained in steel, and it is limited to 0.04% or less because it causes grain boundary corrosion during pickling or impairs hot workability. The preferred P content is 0.01 to 0.04%.

The content of S is 0.002% or less.

S is an inevitable impurity contained in steel, and its content is limited to 20 ppm or less because it segregates at grain boundaries and impairs hot workability.

The content of Ti is 0.15 to 0.3%.

Ti should be added in order to increase the corrosion resistance of the weld, so it is added in an amount of at least 0.15%. However, since Ti combines with C and N to form Ti(C, N) precipitates to lower the amount of solid solution C and N, and Ti(C, N) precipitates hinder the movement of the magnetic domain wall, Ti makes the vibration attenuation ability inferior. Therefore, the content is limited to 0.3% or less.

The content of Nb is 0.15 to 0.3%.

Nb is also an element that is essentially added to increase the corrosion resistance of the weld. When Nb satisfies the appropriate component conditions and heat treatment conditions, fine laves phase precipitates are generated, which helps to improve the vibration attenuation ability. Nb therefore is added in an amount of at least 0.15%. However, since Nb combines with C and N to form Nb(C,N) precipitates to lower the amount of solid solution C and N, and Nb C,N) precipitates hinder the movement of the magnetic domain wall, Nb makes the vibration attenuation ability inferior. Therefore, the content is limited to 0.3% or less.

The content of Cu is 0.15 to 0.3%.

Cu generates fine precipitates by appropriate heat treatment and helps to improve vibration attenuation ability, so it is added in an amount of at least 0.15%. However, if the content of Cu is high, the hot workability at high temperature may be impaired, so the content is limited to 0.3% or less.

The content of Al is 0.01 to 0.05%.

Al combines with N to form AIN precipitates to lower the amount of solid solution N, and because AIN precipitates hinder the movement of the magnetic domain wall, it makes the vibration attenuation ability inferior. In addition, Al is an alloy component that is added as a deoxidizing agent during steelmaking, but when added in a large amount, it exists as non-metallic inclusions and causes sliver defects in the cold-rolled strip, so its content is limited to 0.01 to 0.05%.

The remainder of the ferritic stainless steel except for the above alloying elements is made up of Fe and other inevitable impurities.

The low-Cr ferritic stainless steel according to the invention satisfies Equation (1) below. $\left(Nb+Cu\right) / Ti \geq 1.5$

As the content of Ti increases, the formation of Ti(C,N) precipitates increases to lower the solid solution C and N, and the vibration attenuation ability decreases because the precipitates themselves interfere with the movement of the magnetic domain wall. In order to overcome this, it is necessary to increase the Nb+Cu content so that the vibration attenuating effect by the fine Nb Laves phase precipitate and Cu precipitate should be increased. When the above equation (1) is satisfied together with the above-described alloy component composition, the vibration attenuation ability can be significantly improved compared to the existing one.

The low-Cr ferritic stainless steel according to the invention satisfies Equation (2) below. $Nb + Cu \leq 0.5$

When the content of Nb+Cu becomes higher than necessary, coarsening of precipitates easily occurs. In this case, the coherency between the precipitate and the matrix decreases, and the number of precipitates and the total interface area are reduced, so that the vibration attenuation effect due to the Nb Laves-phase precipitate and the Cu precipitate is difficult to develop. Therefore, the Nb+Cu content is limited to 0.5% or less.

The Nb Laves phase precipitate is Fe₂Nb, and the size of the Nb Laves phase precipitate and the Cu precipitate may be 1 to 200 nm. As described above, when the size of the Nb Laves-phase precipitate and the Cu precipitate are coarse, the number of precipitates is relatively small compared to the fine precipitates, and the coherency between the precipitate and the matrix interface is poor, so that the vibration attenuation effect is small. Therefore, in order to maximize the vibration attenuation ability, it is desirable to control the size of the precipitate to 200 nm or less.

The low-Cr ferritic stainless steel of present invention including 5×10²/ mm² or more of Nb laves phase precipitates and Cu precipitates of 200 nm or less has a vibration attenuation index (Q-1) of 2.0×10⁻⁴ or more at 25°C and 2.5×10⁻⁴ or more at 300°C, which amounts to excellent vibration attenuation.

Next, a method of manufacturing a low-Cr ferritic stainless steel with excellent vibration attenuation ability according to the present disclosure will be described.

The manufacturing method of the low-Cr ferritic stainless steel with excellent vibration attenuation ability of the invention is manufactured into a cold-rolled steel plate through a conventional manufacturing process, and includes cold-rolling annealing a cold-rolled steel plate of the ferritic stainless steel containing the above-described alloy component composition at a temperature of (Ac1-10) °C or less; quenching at 400 to 600°C and maintaining for 5 minutes or more.

For example, the slab including the above-described alloy component composition may be hot-rolled, the hot-rolled steel plate may be annealed, and cold-rolled to form a cold-rolled steel plate.

Cold-rolled steel plate is cold-rolled and annealed in a temperature range below the temperature 10°C lower than the austenite-ferrite transformation temperature (Ac1). Since some austenite phase exists in the Cr content range of the present invention, the annealing temperature is limited to (Ac1-10) °C or less to prevent reverse transformation. Annealing is performed so that C and N are sufficiently dissolved in the matrix within the above temperature range.

In addition, in order to suppress the formation of Cr carbonitrides, quenching is required in a temperature range of 400 to 600°C after cold rolling annealing, and by increasing the number of fine Nb Laves phase precipitates and Cu precipitates through heat treatment maintained in the above temperature range for 5 minutes or more, vibration attenuation ability can be maximized.

At this time, when the Nb+Cu content according to equation (2) exceeds 0.5%, as compared to the Nb Laves phase precipitate and Cu precipitate, which are additionally generated by the heat treatment, the pre-precipitated precipitates are coarsened, so that the total number of precipitates may be reduced. Therefore, when the Nb+Cu content exceeds 0.5%, it is preferable not to perform additional heat treatment after cold rolling annealing.

Hereinafter, it will be described in more detail through a preferred example of the invention.

### Example

The vibration attenuation ability was measured through IMCE's "RFDA LTVP800" equipment. The above equipment generates vibration at a natural frequency by applying a shock of a certain force to a sample of 80 mm (length) * 20 mm (width), and then measures the degree of attenuation of the sound to obtain the vibration attenuation index (Q-1). The higher the vibration attenuation index, the faster the vibration is attenuated. In other words, it has excellent vibration attenuation ability. In the above equipment, the vibration attenuation index can be obtained for a temperature range of 25 ~ 800°C. For each of the final heat-treated alloys, the vibration attenuation index at room temperature (25°C) and 300°C was calculated. The natural frequency was 1 kHz.

The number of Nb Laves phase precipitates and Cu precipitates was measured for only precipitates having a size of 200 nm or less.

**<table 1>**

| | C | N | Si | Mn | Cr | Ti | Nb | Cu | (Nb+Cu) /Ti | (Nb+Cu) |
|---|---|---|---|---|---|---|---|---|---|---|
| Inventive example1 | 0.00 7 | 0.008 | 0.27 | 0.41 | 11.7 | 0.19 | 0.18 | 0.23 | 2.16 | 0.41 |
| Inventive example 2 | 0.00 6 | 0.007 | 0.35 | 0.28 | 12.5 | 0.16 | 0.22 | 0.27 | 3.06 | 0.49 |
| Comparative example1 | 0.00 5 | 0.009 | 0.45 | 0.33 | 10.5 | 0.11 | 0.12 | 0.12 | 2.18 | 0.24 |
| Comparative example 2 | 0.00 8 | 0.006 | 0.29 | 0.29 | 13.1 | 0.38 | 0.34 | 0.32 | 1.74 | 0.66 |
| Comparative example 3 | 0.00 5 | 0.006 | 0.23 | 0.22 | 11.2 | 0.25 | 0.16 | 0.17 | 1.32 | 0.33 |
| Comparative example 4 | 0.00 9 | 0.009 | 0.17 | 0.53 | 11.8 | 0.16 | 0.28 | 0.27 | 3.44 | 0.55 |

**<table 2>**

| | After annealing, maintain 500°C for 5 minutes | Total amount of Nb and Cu precipitates (ea/mm²) | vibration attenuation index (Q-1, ×10⁻⁴) @25°C | vibration attenuation index (Q-1, ×10⁻⁴) @300°C |
|---|---|---|---|---|
| Inventive example 1 | × | 528 | 2.3 | 2.5 |
| | ○ | 679 | 3.1 | 3.3 |
| Inventive example 2 | × | 613 | 2.8 | 3.1 |
| | ○ | 718 | 3.5 | 3.7 |
| Comparative example 1 | × | 289 | 1.1 | 1.2 |
| | ○ | 360 | 1.2 | 1.3 |
| Comparative example 2 | × | 336 | 1.3 | 1.4 |
| | ○ | 435 | 1.5 | 1.6 |
| Comparative example 3 | × | 359 | 1.4 | 1.5 |
| | ○ | 460 | 1.5 | 1.7 |
| Comparative example 4 | × | 410 | 1.6 | 1.6 |
| | ○ | 275 | 1.1 | 1.2 |

FIG. 1 is a graph showing the correlation of the vibration attenuation index according to the number of Nb Laves phase precipitates and Cu precipitates. The results of analyzing the data of the inventive examples and comparative examples of Tables 1 to 2 with reference to FIG. 1 are as follows.

Looking at Invention Examples 1 and 2, by satisfying both the component range of the present invention and Equations (1) and (2), even without heat treatment at 500° C for 5 minutes or more after annealing, the total amount of Nb Laves phase precipitate and Cu precipitate is 500 or more per mm², and at room temperature, the vibration attenuation index (Q-1) was measured to be 2.3×10⁻⁴ or higher. In particular, in the case of performing heat treatment, it was found that the total amount of precipitates increased by 100 to 150 to increase 15 to 30%. Accordingly, the vibration attenuation index (Q-1) was also increased by 20 to 35% and was measured to be 3.1×10⁻⁴ or more.

Comparative Example 1 satisfies Equations (1) and (2), but the content of Ti, Nb, and Cu did not reach 0.15%, so even after annealing and additional heat treatment at 500°C, the total amount of precipitates was as small as 360 /mm². It was found that this was due to insufficient Nb and Cu content for forming the Nb Laves phase precipitate and Cu precipitate.

In Comparative Example 2, the content of Ti, Nb, and Cu all exceeded 0.3%, so that the Nb+Cu value in equation (2) exceeded 0.5%, and accordingly, even after annealing and additional heat treatment at 500°C, the total amount of precipitates did not reach 500 /mm². Equation (1) is satisfactory, but since the content of Ti and Nb is high, forming carbonitrides with C and N, lowering the solid solution C and N, and since the carbonitride itself interferes with the movement of the magnetic domain wall, it was confirmed that the vibration attenuation ability was degraded. In addition, it was estimated that the total amount of precipitates was lower than that of the inventive example as the precipitates became coarse due to the high content of Cu as well as Nb.

Comparative Example 3 satisfies all the component ranges of the present invention including Ti, Nb, and Cu, but does not satisfy Equation (1) due to the high content of Ti compared to Nb+Cu, and accordingly, a large amount of Ti(C,N) carbonitrides was precipitated. FIG. 2 is a photograph showing the distribution of Nb Laves phase precipitates and Cu precipitates at the matrix interface of Comparative Example 3. It can be seen that TiN was generated due to the high Ti content. These TiN precipitates not only lower the solid solution C and N, but also the precipitates themselves hinder the movement of the magnetic domain wall. The vibration attenuation index was also measured to be 1.7×10⁻⁴ or less even after additional heat treatment.

Comparative Example 4 satisfies the component range of the present invention including Ti, Nb, and Cu and equation (1), but does not satisfy Equation (2) due to the high Nb+Cu content. In Comparative Example 4, the content of Nb+Cu was high at 0.55%, so it was estimated that the Nb Laves phase precipitate and the Cu precipitate were coarsened. In particular, as a result of heat treatment at 500°C after annealing, the total amount of precipitates having a size of 200 nm or less was reduced, which was confirmed to be due to the coarsening of the precipitates. When the precipitate becomes coarse, the coherency of the matrix interface and the interface area are lowered, thereby reducing the vibration attenuation effect. After the additional heat treatment of Comparative Example 4, the vibration attenuation index was the lowest despite satisfying the component range of the present invention.

### [Industrial Applicability]

The ferritic stainless steel according to the present invention maximizes vibration attenuation ability by utilizing Nb and Cu fine precipitation phases, thereby securing quietness and durability of vehicle exhaust system parts.

## Claims

1. A low-Cr ferritic stainless steel with excellent vibration attenuation ability, the ferritic stainless steel comprising, in percent % by weight of the entire composition, C: 0.005 to 0.01%, N: 0.005 to 0.01%, Si: 0.1 to 0.9%, Mn: 0.1 to 0.9%, Cr: 9 to 14%, Ni: 0.3% or less, P: 0.04% or less , S: 0.002% or less, Ti: 0.15 to 0.3%, Nb: 0.15 to 0.3%, Cu: 0.15 to 0.3%, Al: 0.01 to 0.05%, the remainder of iron (Fe) and other inevitable impurities;
wherein the content of C + N is less than or equal to 0.02%;
wherein the ferritic stainless steel comprises 5×10²/ mm² or more of Nb laves phase precipitates and Cu precipitates, measured with a method as of description, and
wherein a vibration attenuation index (Q-1) of the stainless steel is 2.0×10⁻⁴ or more at 25°C, 2.5×10⁻⁴ or more at at 300°C, measured with the method as of description,
wherein the ferritic stainless steel satisfies the following Equation (1) $\left(Nb+Cu\right) / Ti \geq 1.5$ Nb, Cu, Ti mean the content % by weight of each element
, wherein the ferritic stainless steel satisfies the following Equation (2) $Nb + Cu \leq 0.5$ Nb, Cu mean the content % by weight) of each element
wherein the Nb Laves phase precipitate is Fe₂Nb, and
the size of the Nb Laves phase precipitate and the Cu precipitate is 1 to 200nm.

2. A manufacturing method of a low-Cr ferritic stainless steel with excellent vibration attenuation ability, according to claim 1, the manufacturing method comprising:
cold-rolling annealing a cold-rolled steel plate of a ferritic stainless steel comprising in percent (%) by weight of the entire composition, C: 0.005 to 0.01%, N: 0.005 to 0.01%, Si: 0.1 to 0.9%, Mn: 0.1 to 0.9%, Cr: 9 to 14%, Ni: 0.3% or less, P: 0.04% or less, S: 0.002% or less, Ti: 0.15 to 0.3%, Nb: 0.15 to 0.3%, Cu: 0.15 to 0.3%, Al: 0.01 to 0.05%, the remainder of iron (Fe) and other inevitable impurities, at a temperature of (Ac1-10)°C or less, wherein the content of C + N is less than or equal to 0.02%; and
quenching at 400 to 600°C and maintaining for 5 minutes or more, thereby producing a low-Cr ferritic stainless steel in which a vibration attenuation index (Q-1) of the stainless steel is 2.0×10⁻⁴ or more at 25°C, 2.5×10⁻⁴ or more at 300°C.
wherein the cold-rolled steel plate satisfies the following Equation (1) $\left(Nb+Cu\right) / Ti \geq 1.5$ Nb, Cu, Ti mean the content % by weight of each element
wherein the cold-rolled steel plate satisfies the following Equation (2) $Nb + Cu \leq 0.5$ Nb, Cu mean the content % by weight of each element

## Patentansprüche

1. Ferritischer Stahl mit niedrigem Cr-Gehalt mit ausgezeichneter Vibrationsdämpfungskapazität, wobei der ferritische Stahl in Gewichtsprozent % der gesamten Zusammensetzung umfasst: C: 0,005 bis 0,01 %, N: 0,005 bis 0,01 %, Si: 0,1 bis 0,9 %, Mn: 0,1 bis 0,9 %, Cr: 9 bis 14 %, Ni: 0,3 % oder weniger, P: 0,04 % oder weniger, S: 0,002 % oder weniger, Ti: 0,15 bis 0,3 %, Nb: 0,15 bis 0,3 %, Cu: 0,15 bis 0,3 %, Al: 0,01 bis 0,05 %, wobei der Rest aus Eisen (Fe) und anderen unvermeidbaren Verunreinigungen besteht;
wobei der Gehalt von C + N kleiner oder gleich 0,02 % ist;
wobei der ferritische Stahl 5×10²/mm² oder mehr Nb-Laves-Phase-Ausscheidungen und Cu-Ausscheidungen umfasst, gemessen mit einem Verfahren gemäß Beschreibung, und wobei ein Vibrationsdämpfungsindex (Q-1) des Edelstahls 2,0×10⁻⁴ oder mehr bei 25 °C, 2,5×10⁻⁴ oder mehr bei 300 °C beträgt, gemessen mit dem Verfahren nach Beschreibung, wobei der ferritische Stahl die folgende Gleichung (1) erfüllt: $\left(Nb+Cu\right) / Ti \geq 1,5$
Nb, Cu, Ti die Gew.-% des Gehalts jeden Elements bedeuten wobei der ferritische Stahl die folgende Gleichung (2) erfüllt: $Nb + Cu \leq 0,5$ Nb, Cu die Gew.-% des Gehalts jeden Elements bedeuten wobei die Nb-Laves-Phase-Ausscheidung Fe₂Nb ist, und die Größe wobei die Nb-Laves-Phase-Ausscheidung und die Cu-Ausscheidung 1 bis 200 nm beträgt.

2. Herstellungsverfahren eines ferritischen Stahls mit niedrigem Cr-Gehalt mit ausgezeichneter Vibrationsdämpfungskapazität nach Anspruch 1,
wobei das Herstellungsverfahren umfasst:
Kaltwalzen und Tempern einer kaltgewalzten Stahlplatte aus ferritischem Stahl, umfassend, in Gewichtsprozent (%) der gesamten Zusammensetzung, C: 0,005 bis 0,01 %, N: 0,005 bis 0,01 %, Si: 0,1 bis 0,9 %, Mn: 0,1 bis 0,9 %, Cr: 9 bis 14 %, Ni: 0,3 % oder weniger, P: 0,04 % oder weniger, S: 0,002 % oder weniger, Ti: 0,15 bis 0,3 %, Nb: 0,15 bis 0,3 %, Cu: 0,15 bis 0,3 %, Al: 0,01 bis 0,05 %, wobei der Rest aus Eisen (Fe) und anderen unvermeidbaren Verunreinigungen besteht, bei einer Temperatur von (Ac1-10) °C oder weniger, wobei der Gehalt von C + N kleiner oder gleich 0,02 % ist; und
Abkühlen bei 400 bis 600 °C und Beibehalten für 5 Minuten oder mehr, dadurch Herstellen eines ferritischen Stahls mit niedrigem Cr-Gehalt, in welchem ein Vibrationsdämpfungsindex (Q-1) des Edelstahls 2,0×10⁻⁴ oder mehr bei 25 °C, 2,5×10⁻⁴ oder mehr bei 300 °C beträgt.
wobei die kaltgewalzte Stahlplatte die folgende Gleichung (1) erfüllt: $\left(Nb+Cu\right) / Ti \geq 1,5$ Nb, Cu, Ti die Gew.-% des Gehalts jeden Elements bedeuten wobei die kaltgewalzte Stahlplatte die folgende Gleichung (2) erfüllt: $Nb + Cu \leq 0 ,5$ Nb, Cu die Gew.-% des Gehalts jeden Elements bedeuten

## Revendications

1. Acier inoxydable ferritique à faible teneur en Cr présentant une excellente capacité d'atténuation des vibrations, l'acier inoxydable ferritique comprenant, en pourcentage % en poids de la composition entière,
C : 0,005 à 0,01 %, N : 0,005 à 0,01 %, Si : 0,1 à 0,9 %, Mn : 0,1 à 0,9 %, Cr : 9 à 14 %, Ni : 0,3 % ou moins, P : 0,04 % ou moins, S : 0,002 % ou moins, Ti : 0,15 à 0,3 %, Nb : 0,15 à 0,3 %, Cu : 0,15 à 0,3 %, Al : 0,01 à 0,05 %, le reste de fer (Fe) et autres impuretés inévitables ;
dans lequel la teneur en C + N est inférieure ou égale à 0,02 % ;
dans lequel l'acier inoxydable ferritique comprend 5×10²/ mm² ou plus de précipités de phase de laves de Nb et de précipités de Cu, mesurés avec un procédé tel que celui de la description, et
dans lequel un indice d'atténuation des vibrations (Q-1) de l'acier inoxydable est de 2,0×10^{~4} ou plus à 25°C, de 2,5×10⁻⁴ ou plus à 300°C, mesuré avec le procédé tel que décrit, dans lequel l'acier inoxydable ferritique satisfait à l'équation (1) suivante $\left(Nb+Cu\right) / Ti \geq 1 ,5$
Nb, Cu, Ti désignent la teneur en % en poids de chaque élément, dans lequel l'acier inoxydable ferritique satisfait à l'équation (2) suivante $Nb + Cu \leq 0,5$
Nb, Cu désignent la teneur en % en poids de chaque élément
dans lequel le précipité de phase de laves de Nb est Fe₂Nb, et
la taille du précipité de phase de laves de Nb et du précipité de Cu est de 1 à 200 nm.

2. Procédé de fabrication d'un acier inoxydable ferritique à faible teneur en Cr ayant une excellente capacité d'atténuation des vibrations, selon la revendication 1,
le procédé de fabrication comprenant :
le recuit de laminage à froid d'une plaque d'acier laminée à froid d'un acier inoxydable ferritique comprenant en pourcentage (%) en poids de la composition entière, C : 0,005 à 0,01 %, N : 0,005 à 0,01 %, Si : 0,1 à 0,9 %, Mn : 0,1 à 0,9 %, Cr : 9 à 14 %, Ni : 0,3 % ou moins, P : 0,04 % ou moins, S : 0,002 % ou moins, Ti : 0,15 à 0,3 %, Nb : 0,15 à 0,3 %, Cu : 0,15 à 0,3 %, Al : 0,01 à 0,05 %, le reste de fer (Fe) et d'autres impuretés inévitables, à une température de (Ac1-10)°C ou moins, dans lequel la teneur en C + N est inférieure ou égale à 0,02 % ; et
la trempe à 400 à 600°C et le maintien pendant 5 minutes ou plus, produisant ainsi un acier inoxydable ferritique à faible teneur en Cr dans lequel un indice d'atténuation des vibrations (Q-1) de l'acier inoxydable est de 2,0×10⁻⁴ ou plus à 25°C, 2,5×10⁻⁴ ou plus à 300°C,
dans lequel la plaque d'acier laminée à froid satisfait à l'équation (1) suivante $\left(Nb+Cu\right) / Ti \geq 1,5$
Nb, Cu, Ti désignent la teneur en % en poids de chaque élément
dans lequel la plaque d'acier laminée à froid satisfait à l'équation (2) suivante $Nb + Cu \leq 0,5$
Nb, Cu désignent la teneur en % en poids de chaque élément.
